



US005248915A

# United States Patent [19]

Tong et al.

[11] Patent Number: 5,248,915  
[45] Date of Patent: Sep. 28, 1993

[54] **ALKOXYSILANE COATING FOR CATHODE RAY TUBES**

4,582,761 4/1986 Liu ..... 428/442  
4,945,282 7/1990 Kawamura et al. ..... 313/479  
5,153,481 10/1992 Matsuda et al. ..... 359/893

[75] Inventors: **Hua-Sou Tong, Arlington Heights; Gregory Prando, Chicago, both of Ill.**

*Primary Examiner*—Michael Lusignan

[73] Assignee: **Zenith Electronics Corporation, Glenview, Ill.**

## [57] ABSTRACT

[21] Appl. No.: 771,079

The present invention is directed to a cathode ray tube (CRT) having a surface with improved antistatic and antiglare properties and to a method for providing such improved properties. In the method of the invention, a solution of an alkoxy silane in a solvent system of an alcohol, chloride ion and water is provided. The solution is applied to the surface of a cathode ray tube to impart antiglare and antistatic properties to the surface. Thereafter, the CRT with the saline applied is cured at an elevated temperature for a period of time sufficient to cause the saline to react and be converted to a siloxane.

[22] Filed: Oct. 2, 1991

32 Claims, 1 Drawing Sheet

[51] Int. Cl.<sup>5</sup> ..... H01J 31/00

[52] U.S. Cl. ..... 313/478; 313/479; 427/64; 427/387; 427/110

[58] Field of Search ..... 313/478, 479; 427/64, 427/66, 110; 422/387

## [56] References Cited

### U.S. PATENT DOCUMENTS

3,689,312 9/1972 Long et al. ..... 117/94  
4,563,612 7/1986 Deal et al. ..... 313/478





*Fig. 1*



*Fig. 2*

## ALKOXYSILANE COATING FOR CATHODE RAY TUBES

### FIELD OF THE INVENTION

The present invention relates generally to a cathode ray tube (CRT) having a coating on the face panel thereof which provides antiglare and antistatic properties. More particularly, the present invention relates to a method for providing an antiglare and antistatic coating on the face panel of CRT's.

### BACKGROUND OF THE INVENTION

Cathode ray tubes are increasingly being used as visual display terminals (VDT's) which are scanned at close range by the human eye. It is desirable to minimize the glare that is reflected from the glass surface of the CRT so as to enable the user to more easily read the graphics and other display characters that are shown on the screen.

Various methods are known for reducing the glare on CRT face panels. U.S. Pat. No. 4,945,282 to Kawamura describes a process for providing antistatic and antiglare properties to the surface of a CRT. The process involves applying a suspension of electroconductive metal oxide particles in an alcoholic solution of alkoxy silane onto the front surface of a CRT. This is followed by heat treatment to the resulting coat to form an antistatic film comprising a transparent electroconductive  $\text{SiO}_2$  coat on the front surface. Antiglare properties are provided by applying a second non-glare film over the electroconductive  $\text{SiO}_2$  coat. The formulation of the non-glare film includes the steps of dispersing fine  $\text{SiO}_2$  particles in an alcoholic solution of alkoxy silane, applying the suspension over the antistatic film which is the transparent substrate formed on the panel and heating the resultant coat to decompose the alkoxy silane to form a thin  $\text{SiO}_2$  film to thereby cover and fix the fine  $\text{SiO}_2$  particles.

U.S. Pat. No. 4,563,612 to Deal, et al. describes a cathode ray tube having an antistatic, glare-reducing coating. The coating has a rough surface which is composed essentially of a silicate material and an inorganic metallic compound. The coating is applied by spraying a solution of a water soluble salt of one or more of a metal selected from platinum, tin, palladium and gold in a lithium stabilized silica sol onto the surface of the cathode ray tube. A solution of lithium, sodium and potassium silicate or an organic silicate, such as tetraethyl orthosilicate may be substituted for the lithium stabilized silica sol.

U.S. Pat. No. 4,582,761 to Liu discloses an aqueous dispersion of polyvinyl acetate for use as a coating on an electronic viewing screen to provide antiglare properties.

U.S. Pat. No. 3,689,312 to Long, et al. is directed to a method for producing a glare-reducing coating on the surface of a cathode ray tube. The method includes the steps of preparing a coating formulation consisting of a solution of a siliceous polymer and an organic polymer in a volatile organic liquid vehicle for the polymers. The solution is then sprayed onto the surface of a cathode ray tube to coat the surface. The cathode ray tube is then baked at a temperature of 100° C to 200° C. to cure the coating.

A cathode ray tube having an antistatic film is disclosed in U.S. Pat. No. 4,785,227 to Matsuda, et al. The antistatic film is applied by dipping the cathode ray tube

into a mixture of tetraethyl silicate, propanol and butanol containing a colloidal solution of metal particles.

It is known to apply a solution of tetrachlorosilane in an anhydrous alcohol to the surface of a CRT heated to 50° C. to 80° C. to reduce glare. The tube surface is then heated to a temperature up to 200° C. for 15-20 minutes to cause polymerization of the silane to a polysiloxane. In this method, the silane solution is sprayed onto the surface of the CRT in the form of discrete island droplets of the solution. A continuous film of the solution must be avoided to provide optimum antiglare properties.

It is also known to apply coatings of lithium silicate onto the surface of a CRT to provide antiglare properties.

While various prior art methods have been proposed for reducing gloss and providing antiglare properties to the surface of a CRT, such methods have not met with complete success. It is important that any coating provided on the surface of the CRT to reduce gloss does not impart undesirable side effects, such as the provision of a mottled or uneven surface. The diffusive reflectivity of the surface imparted by the coating should also not be substantially different than that of the uncoated CRT.

### BRIEF DESCRIPTION OF THE DRAWINGS

The features of the present invention which are believed to be novel are set forth with particularity in the appended claims. The invention, together with further objects and advantages thereof, may best be understood by reference to the following description taken in conjunction with the accompanying drawings, in the figures of which like reference numerals identify like elements, and in which:

FIG. 1 is a cut-away view in perspective of a cabinet that houses a color cathode ray tube, showing certain components, including a front panel, which are the subject of the present invention; and

FIG. 2 is a cross-sectional view, broken away, of the front panel of the cathode ray tube of FIG. 1.

### DESCRIPTION OF THE PREFERRED EMBODIMENT

The invention is useful in cathode ray tubes of various types including home entertainment and medium-resolution and high-resolution types for use in color monitors.

FIG. 1 shows a novel video monitor 10 that houses a color cathode ray tube 12 having a front panel assembly according to the invention. The design of the video monitor is the subject of copending Design Patent application Ser. No. 725,040 of common ownership herewith, now abandoned. The monitor, and the associated tube according to the invention, is notable for the flat imaging area 14 that makes possible the display of images in undistorted form. Imaging area 14 also offers a more efficient use of screen area as the corners are relatively square in comparison with the more rounded corners of the conventional cathode ray tube. The front assembly system comprises the components described in the following paragraphs.

A funnel 22 is shown as being attached to a peripheral sealing area 24 on the inner surface of faceplate 16. A high electrical potential is applied through a high voltage conductor (not shown) attached to an anode button 28 which conducts the potential (the source of which is

a high voltage power supply) through the wall of the funnel 22. The potential may be in the range of 18 to 32 kilovolts, by way of example.

With reference also to FIG. 2, the imaging area 14 includes a glass face panel 16 that may be flat, or alternatively, "substantially flat" in that it may have finite horizontal or vertical radii, by way of example. Face panel 16 is represented as having on its inner surface a centrally disposed electron beam target area 19 on which is disposed at least one pattern of phosphor deposits 20. An electrically conductive screen 21 is depicted schematically as being deposited on and overlaying the pattern of phosphor deposits 20. The electrically conductive screen 21 comprises a film of highly reflective, electrically conductive aluminum disposed on the pattern of phosphor deposits 20 by evaporative means or by hot stamping and having a thickness of about 2000 Angstroms. The novel antiglare-antistatic coating 38 of the invention is formed on the outer surface.

Generally in accordance with the present invention, a solution of an alkoxy silane such as tetraethoxysilane, in a solvent system comprising an alcohol, water and chloride ion is applied to the surface of a cathode ray tube (CRT) to impart antistatic and antiglare properties to the surface of the CRT. The CRT with the silane applied is then cured at an elevated temperature to cause the silane to react in the environment of the solution and to be converted to an adhering coating of a siloxane.

The surface of the CRT is first cleaned with a suitable cleaning agent. Suitable cleaning agents include commercial glass detergent, such as 409 TM, manufactured by The Clorox Co. and Windex TM, manufactured by Drackett Products Co. In one embodiment of the invention, a two-step cleaning process is used to assure adherence of the silane solution. In the first step, the surface of the CRT is rubbed with a suitable particulate substance having a fine particle size in the range of from about 3 to about 12 microns. Suitable particulate substances are metal oxides such as cerium oxide or alumina; volcanic glasses, such as pumice; and friable silicon materials, such as rottenstone. The CRT is then rinsed with water. In the second step, the CRT is cleaned by the application of a commercial glass detergent and is again rinsed with water. The CRT is then dried in air, preferably the use of compressed air.

The chloride ion is provided by adding hydrochloric acid to the alcohol. The chloride ion is present in the solvent system at a level of from about 0.01 to about 1.3 mols of chloride ion per 100 grams of solution. A suitable level of chloride ion can be provided using concentrated hydrochloric acid at a level of from about 1% to about 15%. The silane is preferably present in the solution at a level of from about 0.5 percent to about 50 percent by weight, based on the weight of the alcohol. All percentages used herein are by weight, unless otherwise indicated.

The alcohol for use in the solvent system of the present invention is an aliphatic C<sub>1</sub>-C<sub>4</sub> alcohol. Preferred alcohols are selected from the group consisting of ethanol, propanol and butanol. A particularly preferred alcohol is ethanol.

The amount of water in the solvent system is from about 5% to about 45%. While the water can be present in the solvent system for silanes at a level of up to about 45%, best results in terms of solution stability, gloss reduction and diffusive reflectance are obtained when the water is present at a level of from about 5% to about 25%.

The silane solution is applied to the surface of the cathode ray tube by spraying a fine mist of the solution onto the surface. The surface of the cathode ray tube is preheated prior to the application of the solution to initiate the chemical reaction, which will form silane particles on the surface of panels. The preheated surface also helps to evaporate the alcohol and water and prevents running of the solution. The surface of the cathode ray tube is preferably preheated to a temperature of from about 90° C. to about 120° C. The fine mist of the silane solution is applied so as to form a plurality of discrete droplets uniformly over the surface of the CRT.

In the method of the invention, it is important that the solution drops which are sprayed onto the surface of the CRT have a particle size in the range of from about 0.3 to about 0.5 microns at the point of arrival at the surface of the CRT. The desired solution drop size can be attained by use of a compressed air spray gun having a fluid nozzle orifice of from about 0.05 to about 0.13 cm and which is operated at an air pressure of 30-60 psig, a fluid pressure of 5-15 psig and a distance of spray gun to CRT surface of 18-25 cm. The solution is preferably applied to the surface of the cathode ray tube at a level sufficient to provide from about 0.3 to about 1.2 milligrams of the silane per square centimeter of the surface area.

A single pass of a spray gun over the surface of the front panel of the cathode ray tube may not result in the application of the desired amount of the solution of the silane. The solution may be applied in multiple layers such as by repeatedly passing a spray gun over the surface of the cathode ray tube. The cathode ray tube is preferably preheated to a temperature in the range of from about 90° C. to about 120° C. prior to the first spray pass and the remaining spray passes are made prior to any substantial cooling of the surface. In an important embodiment of the invention, from about 3 to about 12 spray passes of the solution are applied.

After the solution of silane is applied, the cathode ray tube may be cured at an elevated temperature for a period of time sufficient to convert the silane to siloxane. Suitable temperature and time conditions are a temperature of from about 120° C. to about 200° C. for a period of from about 0.1 hour to about 2 hours. Curing at an elevated temperature is not essential and curing may be effected at ambient temperature.

The following examples further illustrate various features of the present invention, but are intended to in no way limit the scope of the invention which is defined in the appended claims.

#### EXAMPLE 1

A solution of tetraethoxysilane was prepared having the following components at the indicated levels.

| Component         | Weight Percent |
|-------------------|----------------|
| Tetraethoxysilane | 3              |
| Water             | 20             |
| Hydrochloric Acid | 3-15           |
| Ethanol           | balance        |

A CRT was cleaned by buffing with a buffing compound, which is a uniform paste having 1 part by weight of cerium oxide having a particle size in the range of 3 to 12 microns, 1 part by weight of Syloid 244 (Davidson), 1 part by weight mineral spirits, 1 part by weight

methylene chloride and 1 part by weight xylene. This is followed by rinsing with tap water, cleaning with a commercial glass detergent (Windex™ manufactured by Drackett Products Co., Cincinnati, Oh.), rinsing again with tap water and drying by directing a stream of compressed air over the surface of the CRT.

Several of the above silane solutions with various levels of hydrochloric acid were sprayed onto the panel surface of cleaned cathode ray tubes which had been preheated to a temperature of 90° C. The solvent and water were flashed from the surface of the face panel to provide a coating of silane. Spraying was accomplished by use of a compressed air spray gun having a nozzle orifice of 0.07 cm, and operated at an air pressure of 50 psig and a fluid pressure of 10 psig. The spray gun was moved back and forth over the surface of the CRT from a distance of 21 cm. Five passes of the spray gun were used to deposit a coating of 0.5 mg of silane per cm<sup>2</sup> of surface area. The cathode ray tubes were then cured at a temperature of 150° C., 175° C., 200° C. or 225° C. for 20

thin layer of silicon oxide. The gloss reduction of the face panel without coating was 92%. After coating with the coating composition of the invention, the gloss reduction was 56%.

An important function of the present invention is to provide antistatic properties for a CRT surface. CRT's having the above silane composition applied thereto, were tested for antistatic properties using an electrostatic meter. For this test, the CRT was turned on, which immediately imparted a 25 KeV charge on the surface of the tube. The meter was held two inches from the surface of the tube. While the CRT remained on the CRT surface was grounded and the time in seconds for the surface charge to decay from 25 KeV to 0 KeV was measured. The ground was then removed and the CRT was turned off. The time in seconds for the charge to decay from 25 KeV to 0 KeV was again measured. The results for several test runs are set forth below in Tables 1 through 5. The lower the time required for decay the better for these tests.

TABLE 1

| TRIAL | TIME ELAPSE FOR TES/20% WATER/ETOH + 3% HCl |    |    |    |     |     |         |    |    |    |    |    |     |         |
|-------|---------------------------------------------|----|----|----|-----|-----|---------|----|----|----|----|----|-----|---------|
|       | ON                                          |    |    |    | OFF |     |         |    |    |    |    |    |     |         |
| TRIAL | 5K                                          | 4K | 3K | 2K | 1K  | .5K | 0       | 5K | 4K | 3K | 2K | 1K | .5K | 0       |
| 1     | 3                                           | 4  | 5  | 6  | 9   | 12  | 26      | 4  | 5  | 6  | 8  | 11 | 16  | 45(.1K) |
| 2     | 3                                           | 4  | 5  | 6  | 9   | 12  | 34      | 4  | 5  | 6  | 8  | 11 | 16  | 38(.1K) |
| 3     | 3                                           | 4  | 5  | 6  | 9   | 12  | 24(.1K) | 4  | 5  | 6  | 8  | 11 | 17  | 43(.1K) |
| 4     | 3                                           | 4  | 5  | 6  | 9   | 12  | 28      | 4  | 5  | 6  | 8  | 11 | 17  | 43(.1K) |

TABLE 2

| TRIAL | TIME ELAPSE FOR TES/20% WATER/ETOH + 6% HCl |    |    |    |     |     |    |    |    |    |    |    |     |         |
|-------|---------------------------------------------|----|----|----|-----|-----|----|----|----|----|----|----|-----|---------|
|       | ON                                          |    |    |    | OFF |     |    |    |    |    |    |    |     |         |
| TRIAL | 5K                                          | 4K | 3K | 2K | 1K  | .5K | 0  | 5K | 4K | 3K | 2K | 1K | .5K | 0       |
| 1     | 2                                           | 3  | 4  | 5  | 6   | 8   | 19 | 2  | 3  | 4  | 5  | 8  | 12  | 31(.1K) |
| 2     | 2                                           | 3  | 4  | 5  | 6   | 8   | 22 | 2  | 3  | 4  | 5  | 8  | 12  | 29(.1K) |
| 3     | 2                                           | 3  | 4  | 5  | 6   | 8   | 26 | 2  | 3  | 5  | 6  | 9  | 14  | 32(.2K) |
| 4     | 2                                           | 3  | 4  | 5  | 6   | 9   | 30 | 2  | 3  | 4  | 5  | 8  | 12  | 28(.1K) |

TABLE 3

| TRIAL | TIME ELAPSE FOR TES/20% WATER/ETOH + 9% HCl |    |    |    |     |     |         |    |    |    |    |    |     |          |
|-------|---------------------------------------------|----|----|----|-----|-----|---------|----|----|----|----|----|-----|----------|
|       | ON                                          |    |    |    | OFF |     |         |    |    |    |    |    |     |          |
| TRIAL | 5K                                          | 4K | 3K | 2K | 1K  | .5K | 0       | 5K | 4K | 3K | 2K | 1K | .5K | 0        |
| 1     | 14                                          | 18 | 22 | 28 | 41  | 54  | 85(.2K) | 17 | 21 | 26 | 34 | 49 | 74  | 160(.2K) |
| 2     | 15                                          | 18 | 23 | 29 | 41  | 54  | 80(.2K) | 17 | 21 | 26 | 33 | 48 | 71  | 100(.3K) |
| 3     | 15                                          | 18 | 23 | 29 | 41  | 54  | 80(.2K) | 17 | 21 | 26 | 33 | 48 | 71  | 100(.3K) |
| 4     | 15                                          | 18 | 22 | 29 | 40  | 54  | 76(.2K) | 17 | 21 | 26 | 34 | 50 | 76  | 129(.3K) |

TABLE 4

| TRIAL | TIME ELAPSE FOR TES/20% WATER/ETOH + 12% HCl |    |    |    |     |     |    |    |    |    |    |    |     |         |
|-------|----------------------------------------------|----|----|----|-----|-----|----|----|----|----|----|----|-----|---------|
|       | ON                                           |    |    |    | OFF |     |    |    |    |    |    |    |     |         |
| TRIAL | 5K                                           | 4K | 3K | 2K | 1K  | .5K | 0  | 5K | 4K | 3K | 2K | 1K | .5K | 0       |
| 1     | 1                                            | 2  | 3  | 4  | 5   | 7   | 14 | 2  | 3  | 4  | 5  | 7  | 10  | 33(.1K) |
| 2     | 1                                            | 2  | 3  | 4  | 5   | 7   | 14 | 2  | 3  | 4  | 5  | 8  | 13  | 54(.2K) |
| 3     | 1                                            | 2  | 3  | 4  | 5   | 7   | 14 | 2  | 3  | 4  | 5  | 8  | 13  | 55(.2K) |
| 4     | 1                                            | 2  | 3  | 4  | 5   | 7   | 14 | 2  | 3  | 4  | 5  | 8  | 14  | 60(.2K) |

a period of twenty minutes. The resulting coating was a

TABLE 5

| TRIAL | TIME ELAPSE FOR TES/20% WATER/ETOH + 15% HCl |    |    |    |     |     |         |    |    |    |    |    |     |         |
|-------|----------------------------------------------|----|----|----|-----|-----|---------|----|----|----|----|----|-----|---------|
|       | ON                                           |    |    |    | OFF |     |         |    |    |    |    |    |     |         |
| TRIAL | 5K                                           | 4K | 3K | 2K | 1K  | .5K | 0       | 5K | 4K | 3K | 2K | 1K | .5K | 0       |
| 1     | 3                                            | 4  | 5  | 6  | 9   | 12  | 35(.1K) | 4  | 5  | 6  | 8  | 11 | 17  | 47(.2K) |
| 2     | 3                                            | 4  | 5  | 6  | 8   | 11  | 22      | 4  | 5  | 6  | 7  | 11 | 17  | 35(.2K) |
| 3     | 3                                            | 4  | 5  | 6  | 8   | 11  | 23      | 4  | 5  | 6  | 7  | 10 | 15  | 34(.1K) |

TABLE 5-continued

| TRIAL | TIME ELAPSE FOR TES/20% WATER/ETOH + 15% HCl |    |    |    |     |     |   |    |    |    |    |    |     |         |
|-------|----------------------------------------------|----|----|----|-----|-----|---|----|----|----|----|----|-----|---------|
|       | ON                                           |    |    |    | OFF |     |   |    |    |    |    |    |     |         |
|       | 5K                                           | 4K | 3K | 2K | 1K  | .5K | 0 | 5K | 4K | 3K | 2K | 1K | .5K | 0       |
| 4     | 4                                            | 5  | 6  | 11 | 13  | 29  |   | 4  | 5  | 6  | 77 | 10 | 15  | 34(.1K) |

It can readily be seen that the silane coating of the invention provides exceptional antistatic properties.

10

and ethanol provides upper antistatic properties as compared to a solvent system which does to include water.

## EXAMPLE 2

Several solutions of tetraethoxysilane in ethyl alcohol were prepared. The solutions had 3% of tetraethoxysilane and either 3% or 6% of hydrochloric acid as indicated in the headings of Tables 6 and 7 hereinbelow. CRT's were measured as described in Example 1. The result are set forth in Tables 6 and 7.

15

Further coating compositions containing 3% tetraethoxysilane, 20% water, ethanol and various levels of either nitric acid or acetic acid. CRT's were coated with these solutions and the antistatic properties were measured as described in Example 1. The results are set forth in Tables 8 through 17 hereinbelow. The designa-

TABLE 6

| TRIAL | TES + 3 WT % HCl - CURING AT 125° C. FOR 20 MINUTES |    |    |    |     |     |    |    |    |    |    |    |     |         |
|-------|-----------------------------------------------------|----|----|----|-----|-----|----|----|----|----|----|----|-----|---------|
|       | ON                                                  |    |    |    | OFF |     |    |    |    |    |    |    |     |         |
|       | 5K                                                  | 4K | 3K | 2K | 1K  | .5K | 0  | 5K | 4K | 3K | 2K | 1K | .5K | 0       |
| 1     | 4                                                   | 5  | 7  | 10 | 15  | 21  | 29 | 4  | 5  | 7  | 10 | 17 | 29  | 60(.2K) |
| 2     | 4                                                   | 5  | 7  | 9  | 14  | 20  | 30 | 4  | 5  | 7  | 10 | 16 | 28  | 60(.2K) |
| 3     | 4                                                   | 5  | 7  | 9  | 14  | 20  | 28 | 4  | 5  | 7  | 10 | 19 | 45  | 90(.3K) |
| 4     | 4                                                   | 5  | 7  | 9  | 14  | 20  | 28 | 4  | 5  | 7  | 9  | 15 | 24  | 57(.1K) |

TABLE 7

| TRIAL | TES + 6 WT % HCl - CURING AT 125° C. FOR 20 MINUTES |    |    |    |     |     |          |    |    |    |    |    |     |          |
|-------|-----------------------------------------------------|----|----|----|-----|-----|----------|----|----|----|----|----|-----|----------|
|       | ON                                                  |    |    |    | OFF |     |          |    |    |    |    |    |     |          |
|       | 5K                                                  | 4K | 3K | 2K | 1K  | .5K | 0        | 5K | 4K | 3K | 2K | 1K | .5K | 0        |
| 1     | 13                                                  | 16 | 20 | 25 | 36  | 48  | 66(.2K)  | 16 | 19 | 24 | 32 | 52 | 94  | 180(.3K) |
| 2     | 13                                                  | 16 | 20 | 26 | 37  | 50  | 81(.2K)  | 16 | 19 | 24 | 32 | 52 | 95  | 180(.3K) |
| 3     | 21                                                  | 26 | 31 | 40 | 57  | 75  | 120(.2K) | 16 | 20 | 24 | 32 | 52 | 98  | 190(.3K) |
| 4     | 21                                                  | 26 | 31 | 40 | 57  | 75  | 120(.2K) | 16 | 20 | 24 | 32 | 52 | 89  | 170(.3K) |

A comparison of Tables 6 and 7 with Tables 1 and 2 shows that the use of a solvent system comprising water

tion "NM" in the tables means that no perceptible movement of the meter needle from the midpoint was observed for 5 minutes.

TABLE 8

| TRIAL | TIME ELAPSE FOR TES/20% WATER/ETOON + 3% NITRIC ACID |    |    |    |    |     |    |     |    |    |    |    |     |    |
|-------|------------------------------------------------------|----|----|----|----|-----|----|-----|----|----|----|----|-----|----|
|       | ON                                                   |    |    |    |    |     |    | OFF |    |    |    |    |     |    |
|       | 5K                                                   | 4K | 3K | 2K | 1K | .5K | 0  | 5K  | 4K | 3K | 2K | 1K | .5K | 0  |
| 1     | NM                                                   | NM | NM | NM | NM | NM  | NM | NM  | NM | NM | NM | NM | NM  | NM |
| 2     | NM                                                   | NM | NM | NM | NM | NM  | NM | NM  | NM | NM | NM | NM | NM  | NM |
| 3     | NM                                                   | NM | NM | NM | NM | NM  | NM | NM  | NM | NM | NM | NM | NM  | NM |
| 4     | NM                                                   | NM | NM | NM | NM | NM  | NM | NM  | NM | NM | NM | NM | NM  | NM |

TABLE 9

| TRIAL | TIME ELAPSE FOR TES/20% WATER/ETOH + % NITRIC ACID |    |     |     |     |          |   |     |     |     |      |     |          |   |
|-------|----------------------------------------------------|----|-----|-----|-----|----------|---|-----|-----|-----|------|-----|----------|---|
|       | ON                                                 |    |     |     |     |          |   | OFF |     |     |      |     |          |   |
|       | 5K                                                 | 4K | 3K  | 2K  | 1K  | .5K      | 0 | 5K  | 4K  | 3K  | 2K   | 1K  | .5K      | 0 |
| 1     | 84                                                 | 89 | 120 | 155 | 237 | 300(.8K) | — | 89  | 105 | 125 | 158  | 219 | 300      | — |
| 2     | 81                                                 | 93 | 116 | 149 | 220 | 300(.6K) | — | 89  | 105 | 127 | 160  | 221 | 300      | — |
| 3     | 81                                                 | 96 | 117 | 150 | 222 | 300(.6K) | — | 89  | 104 | 127 | 159  | 221 | 300      | — |
| 4     | 78                                                 | 94 | 117 | 146 | 206 | 300      | — | 92  | 110 | 132 | 1666 | 238 | 300(.6K) | — |

TABLE 10

| TRIAL | TIME ELAPSE FOR TES/20% WATER/ETOH + 9% NITRIC ACID |     |     |     |           |     |     |     |     |     |           |    |     |   |
|-------|-----------------------------------------------------|-----|-----|-----|-----------|-----|-----|-----|-----|-----|-----------|----|-----|---|
|       | ON                                                  |     |     |     |           |     |     | OFF |     |     |           |    |     |   |
|       | 5K                                                  | 4K  | 3K  | 2K  | 1K        | .5K | 0   | 5K  | 4K  | 3K  | 2K        | 1K | .5K | 0 |
| 1     | 123                                                 | 148 | 184 | 249 | 300(1.6K) | —   | 135 | 160 | 195 | 252 | 300(1.4K) | —  | —   | — |
| 2     | 122                                                 | 150 | 180 | 250 | 300(1.7K) | —   | 133 | 158 | 193 | 250 | 300(1.4K) | —  | —   | — |
| 3     | 113                                                 | 131 | 167 | 240 | 300(1.8K) | —   | 124 | 150 | 187 | 242 | 300(1.5K) | —  | —   | — |
| 4     | 111                                                 | 139 | 180 | 260 | 300(1.8K) | —   | 131 | 158 | 198 | 260 | 300(1.7K) | —  | —   | — |

TABLE 11

| TRIAL | ON |    |    |    |     |     |          | OFF |    |    |    |     |     |          |
|-------|----|----|----|----|-----|-----|----------|-----|----|----|----|-----|-----|----------|
|       | 5K | 4K | 3K | 2K | 1K  | .5K | 0        | 5K  | 4K | 3K | 2K | 1K  | .5K | 0        |
| 1     | 37 | 44 | 55 | 73 | 102 | 141 | 240(.2K) | 40  | 49 | 59 | 78 | 114 | 160 | 230(.2K) |
| 2     | 39 | 46 | 58 | 75 | 109 | 159 | 300(.4K) | 40  | 49 | 60 | 77 | 110 | 150 | 212(.2K) |
| 3     | 37 | 46 | 58 | 75 | 109 | 159 | 300(.4K) | 39  | 47 | 58 | 74 | 105 | 144 | 200(.2K) |
| 4     | 35 | 41 | 52 | 68 | 101 | 139 | 230(.3K) | 39  | 47 | 58 | 75 | 110 | 155 | 200(.2K) |

TABLE 12

| TRIAL | ON |    |    |     |         |     |   | OFF |    |     |     |     |     |          |
|-------|----|----|----|-----|---------|-----|---|-----|----|-----|-----|-----|-----|----------|
|       | 5K | 4K | 3K | 2K  | 1K      | .5K | 0 | 5K  | 4K | 3K  | 2K  | 1K  | .5K | 0        |
| 1     | 59 | 75 | 98 | 139 | 300(1K) |     |   | 67  | 81 | 102 | 132 | 192 | 260 | 300(.4K) |
| 2     | 59 | 72 | 93 | 130 | 195     |     |   | 69  | 84 | 107 | 138 | 200 | 288 |          |
| 3     | 56 | 70 | 90 | 126 | 199     |     |   | 68  | 83 | 106 | 136 | 196 | 265 | 300(.4K) |
| 4     | 58 | 72 | 92 | 125 | 195     |     |   | 69  | 84 | 106 | 140 | 202 | 291 |          |

TABLE 13

| TRIAL | ON  |           |    |    |    |     |    | OFF |    |    |    |    |     |    |
|-------|-----|-----------|----|----|----|-----|----|-----|----|----|----|----|-----|----|
|       | 5K  | 4K        | 3K | 2K | 1K | .5K | 0  | 5K  | 4K | 3K | 2K | 1K | .5K | 0  |
| 1     | 250 | 300(4.2K) | NM | NM | NM | NM  | NM | NM  | NM | NM | NM | NM | NM  | NM |
| 2     | NM  | NM        | NM | NM | NM | NM  | NM | NM  | NM | NM | NM | NM | NM  | NM |
| 3     | NM  | NM        | NM | NM | NM | NM  | NM | NM  | NM | NM | NM | NM | NM  | NM |
| 4     | NM  | NM        | NM | NM | NM | NM  | NM | NM  | NM | NM | NM | NM | NM  | NM |

TABLE 14

| TRIAL | ON |    |    |    |    |     |    | OFF |    |    |    |    |     |    |
|-------|----|----|----|----|----|-----|----|-----|----|----|----|----|-----|----|
|       | 5K | 4K | 3K | 2K | 1K | .5K | 0  | 5K  | 4K | 3K | 2K | 1K | .5K | 0  |
| 1     | NM | NM | NM | NM | NM | NM  | NM | NM  | NM | NM | NM | NM | NM  | NM |
| 2     | NM | NM | NM | NM | NM | NM  | NM | NM  | NM | NM | NM | NM | NM  | NM |
| 3     | NM | NM | NM | NM | NM | NM  | NM | NM  | NM | NM | NM | NM | NM  | NM |
| 4     | NM | NM | NM | NM | NM | NM  | NM | NM  | NM | NM | NM | NM | NM  | NM |

TABLE 15

| TRIAL | ON |    |    |    |    |     |    | OFF |    |    |    |    |     |    |
|-------|----|----|----|----|----|-----|----|-----|----|----|----|----|-----|----|
|       | 5K | 4K | 3K | 2K | 1K | .5K | 0  | 5K  | 4K | 3K | 2K | 1K | .5K | 0  |
| 2     | NM | NM | NM | NM | NM | NM  | NM | NM  | NM | NM | NM | NM | NM  | NM |
| 3     | NM | NM | NM | NM | NM | NM  | NM | NM  | NM | NM | NM | NM | NM  | NM |
| 4     | NM | NM | NM | NM | NM | NM  | NM | NM  | NM | NM | NM | NM | NM  | NM |

TABLE 15

| TRIAL | ON |    |    |    |    |     |    | OFF |    |    |    |    |     |    |
|-------|----|----|----|----|----|-----|----|-----|----|----|----|----|-----|----|
|       | 5K | 4K | 3K | 2K | 1K | .5K | 0  | 5K  | 4K | 3K | 2K | 1K | .5K | 0  |
| 2     | NM | NM | NM | NM | NM | NM  | NM | NM  | NM | NM | NM | NM | NM  | NM |
| 3     | NM | NM | NM | NM | NM | NM  | NM | NM  | NM | NM | NM | NM | NM  | NM |
| 4     | NM | NM | NM | NM | NM | NM  | NM | NM  | NM | NM | NM | NM | NM  | NM |

TABLE 15

| TRIAL | ON |    |    |    |    |     |    | OFF |    |    |    |    |     |    |
|-------|----|----|----|----|----|-----|----|-----|----|----|----|----|-----|----|
|       | 5K | 4K | 3K | 2K | 1K | .5K | 0  | 5K  | 4K | 3K | 2K | 1K | .5K | 0  |
| 2     | NM | NM | NM | NM | NM | NM  | NM | NM  | NM | NM | NM | NM | NM  | NM |
| 3     | NM | NM | NM | NM | NM | NM  | NM | NM  | NM | NM | NM | NM | NM  | NM |
| 4     | NM | NM | NM | NM | NM | NM  | NM | NM  | NM | NM | NM | NM | NM  | NM |

From the foregoing example switch nitric acid and acetic acid, it is apparent the the improved antistatic properties provided by the use of hydrochloric acid and water are not related to reducing the pH with an acid.

While not wishing to be could by any theory, it is believed that the chloride ion is highly hygroscopic and

interacts with moisture from ambient air on the surface of the CRT to provide reduced antistatic properties.

What is claimed is:

1. A method for improving the antistatic and anti-glare properties of the surface of a cathode ray tube comprising:

- (a) providing a solution of an alkoxy silane in a solvent system comprising an alcohol, chloride ion from hydrochloric acid which is present at a level of from about 1% to about 15% and water,
- (b) spraying droplets of said solution onto the surface of a cathode ray tube, and
- (c) curing said silane on said cathode ray tube in a curing step for a period of time sufficient to convert said silane to a siloxane on the surface of said cathode ray tube.

2. A method in accordance with claim 1 wherein said surface of said cathode ray tube is preheated prior to application of said solution.

3. A method in accordance with claim 2 wherein said cathode ray tube is preheated to a temperature in the range of from about 70° C. to about 120° C. prior to applying said solution.

4. A method in accordance with claim 1 wherein said curing of said cathode ray tube is at an elevated temperature of from ambient to about 200° C. for a period of from about 0.1 hour to about 2 hours.

5. A method in accordance with claim 1 wherein said silane is present on the surface of said cathode ray tube at a level of from about 0.3 to 1.2 milligrams per square centimeter of said surface area of said cathode ray tube.

6. A method in accordance with claim 1 wherein said solution is applied by spraying a fine mist of said solution onto said surface.

7. A method in accordance with claim 1 wherein said solution is applied to said surface of said cathode ray tube by multiple spray passes.

8. A method in accordance with claim 7 wherein from 3 to 12 spray passes are used to apply said solution.

9. A method in accordance with claim 1 wherein said silane is present in said solution at a level of from about 0.5 percent to about 50 percent, based on the weight of said solution.

10. A method in accordance with claim 1 wherein said silane is tetraethoxysilane.

11. A method in accordance with claim 1 wherein hydrochloric acid is present in said solution at a level sufficient to provide from about 0.01 to about 1.3 mols of chloride ion per 100 grams of solution.

12. A method in accordance with claim 1 wherein said alcohol is a C<sub>1</sub>-C<sub>4</sub> aliphatic alcohol.

13. A method in accordance with claim 12 wherein said alcohol is ethanol.

14. A method in accordance with claim 12 wherein said alcohol is propanol.

15. A method in accordance with claim 1 wherein said solution droplets have a diameter of from about 0.3 to about 0.5 microns.

16. A method in accordance with claim 1 wherein said alkoxy silane is tetraethoxysilane which is present in said solution at a level of from about 0.5% to about 50%, based on the weight of said solvent systems, said water is present in said solvent system at a level of about 5% to 45%, said hydrochloric acid is present at a level

of from about 1% to about 15% and said alcohol provides the balance of said solution.

17. A cathode ray tube having a surface with reduced gloss comprising a cathode ray tube having a coating on the surface thereof, said coating being provided by spraying fine droplets of a solution of an alkoxy silane in a solvent system comprising an alcohol, chloride ion from hydrochloric acid which is present at a level of from about 1% to about 15% and water onto the surface of said CRT and curing the silane for a period of time sufficient to convert said silane to a siloxane coating on the surface of said cathode ray tube, said siloxane coating having a uniform, fine texture.

18. A cathode ray tube in accordance with claim 17 wherein said surface of said cathode ray tube is preheated prior to application of said solution.

19. A cathode ray tube in accordance with claim 17 wherein said cathode ray tube is preheated to a temperature in the range of from about 70° C. to about 120° C. prior to applying said solution.

20. A cathode ray tube in accordance with claim 17 wherein said curing of said cathode ray tube is at an elevated temperature from ambient to about 200° C. for a period of from about 0.1 hour to about 2 hours.

21. A cathode ray tube in accordance with claim 17 wherein said silane is present on the surface of said cathode ray tube at a level of from about 0.3 to about 1.2 milligrams per square centimeter of said surface area of said cathode ray tube.

22. A cathode ray tube in accordance with claim 17 wherein said solution is applied by spraying a fine mist of said solution onto said surface.

23. A cathode ray tube in accordance with claim 17 wherein said solution is applied to said surface of said cathode ray tube by multiple spray passes.

24. A cathode ray tube in accordance with claim 23 wherein from 3 to 12 spray passes are used to apply said solution.

25. A cathode ray tube in accordance with claim 17 wherein said silane is present in said solution at a level of from about 0.5% to about 50%, based on the weight of said solution.

26. A cathode ray tube in accordance with claim 17 wherein said silane is tetraethoxysilane.

27. A cathode ray tube in accordance with claim 17 wherein hydrochloric acid is present in said solution at a level sufficient to provide from about 0.01 to about 1.3 mols of chloride ion per 100 grams of solution.

28. A cathode ray tube in accordance with claim 17 wherein said alcohol is a C<sub>1</sub>-C<sub>4</sub> aliphatic alcohol.

29. A cathode ray tube in accordance with claim 28 wherein said alcohol is ethanol.

30. A cathode ray tube in accordance with claim 28 wherein said alcohol is propanol.

31. A cathode ray tube in accordance with claim 17 wherein said solution droplets have a diameter of from about 0.3 to about 0.5 microns.

32. A cathode ray tube in accordance with claim 17 wherein said alkoxy silane is tetraethoxysilane which is present in said solution at a level of from about 0.5% to about 50%, based on the weight of said solvent system, said water is present in said solvent system at a level of from 5% to 45%, said hydrochloric acid is present at a level of from about 1% to about 15% and said alcohol provides the balance of said solution.

\* \* \* \* \*